



US010273585B2

(12) **United States Patent**  
**Crondahl et al.**

(10) **Patent No.:** US 10,273,585 B2  
(45) **Date of Patent:** Apr. 30, 2019

(54) **CATHODIC PROTECTION FOR WOOD VENEER DRYERS AND METHOD FOR REDUCING CORROSION OF WOOD VENEER DRYERS**

(71) Applicant: **Westmill Industries Ltd.**, Aldergrove (CA)

(72) Inventors: **Michael Crondahl**, Mission (CA); **Christian Gollmann**, Eugene, OR (US)

(73) Assignee: **Westmill Industries Ltd.**, Aldergrove (CA)

(\*) Notice: Subject to any disclaimer, the term of this patent is extended or adjusted under 35 U.S.C. 154(b) by 232 days.

(21) Appl. No.: **14/736,099**

(22) Filed: **Jun. 10, 2015**

(65) **Prior Publication Data**

US 2016/0362797 A1 Dec. 15, 2016

(51) **Int. Cl.**

**C23F 13/06** (2006.01)  
**C23F 13/04** (2006.01)

(Continued)

(52) **U.S. Cl.**

CPC ..... **C23F 13/06** (2013.01); **C23F 13/04** (2013.01); **C23F 13/16** (2013.01); **F26B 5/16** (2013.01);

(Continued)

(58) **Field of Classification Search**

CPC ..... C23F 13/02; C23F 13/04; C23F 13/08; C23F 13/10; C23F 13/12-13/14;

(Continued)

(56) **References Cited**

U.S. PATENT DOCUMENTS

1,739,766 A 12/1929 Morris  
2,706,342 A \* 4/1955 Willis ..... F26B 7/00  
34/350

(Continued)

FOREIGN PATENT DOCUMENTS

DE 2217715 A \* 4/1971 ..... C23F 13/04  
DE 20 2012 010 945.6 1/2013

(Continued)

OTHER PUBLICATIONS

Beckley (Insulated Aluminum Panels for Dry Kiln Walls and Roofs, 1957, pp. 33-41, [http://ir.library.oregonstate.edu/xmlui/bitstream/handle/1957/5887/Insulated\\_Aluminum\\_ocr.pdf](http://ir.library.oregonstate.edu/xmlui/bitstream/handle/1957/5887/Insulated_Aluminum_ocr.pdf)).\*

(Continued)

*Primary Examiner* — Alexander W Keeling

(74) *Attorney, Agent, or Firm* — Oyen Wiggs Green & Mutala LLP

(57) **ABSTRACT**

A cathodic protection system for use with a wood veneer dryer is provided. The system includes a DC power supply and an anode mounted inside the dryer in a position to be electrolytically coupled to metallic structures or surfaces inside the dryer when an electrolytic medium is present inside the dryer. The electrolytic medium comprises a high-humidity atmosphere. A method for reducing the corrosion of metallic structures or surfaces inside the dryer is further provided. The method comprises mounting an anode inside the dryer in a position to be electrolytically coupled to the metallic structures or surfaces inside the dryer when an electrolytic medium is present. Wood veneer is conveyed through the dryer and heated to a temperature sufficient to produce a high-humidity atmosphere inside the dryer. A controlled amount of current is supplied by the DC power supply to electrolytically couple the anode to the metallic structures or surfaces.

**24 Claims, 4 Drawing Sheets**



|      |                                       |                                                                                                                             |               |         |                 |            |  |
|------|---------------------------------------|-----------------------------------------------------------------------------------------------------------------------------|---------------|---------|-----------------|------------|--|
| (51) | <b>Int. Cl.</b>                       |                                                                                                                             |               |         |                 |            |  |
|      | <i>C23F 13/16</i>                     | (2006.01)                                                                                                                   | 3,350,288 A   | 10/1967 | Almar-Naess     |            |  |
|      | <i>F26B 21/00</i>                     | (2006.01)                                                                                                                   | 3,379,629 A   | 4/1968  | Banks et al.    |            |  |
|      | <i>F26B 5/16</i>                      | (2006.01)                                                                                                                   | 3,585,734 A   | 6/1971  | Barton et al.   |            |  |
|      | <i>C23F 13/14</i>                     | (2006.01)                                                                                                                   | 4,621,669 A   | 11/1986 | Kivimaa         |            |  |
| (52) | <b>U.S. Cl.</b>                       |                                                                                                                             | 5,340,455 A * | 8/1994  | Kroon .....     | C23F 13/06 |  |
|      | CPC .....                             | <i>F26B 21/00</i> (2013.01); <i>C23F 13/14</i> (2013.01); <i>C23F 2213/30</i> (2013.01); <i>F26B 2200/12</i> (2013.01)      | 204/196.3     |         |                 | 204/196.3  |  |
| (58) | <b>Field of Classification Search</b> |                                                                                                                             | 5,954,938 A * | 9/1999  | Takahashi ..... | C23F 13/04 |  |
|      | CPC .....                             | <i>C23F 13/16</i> ; <i>C23F 13/18</i> ; <i>C23F 13/22</i> ; <i>C23F 2213/10</i> ; <i>C23F 2213/30</i> ; <i>C23F 2213/31</i> | 204/196.11    |         |                 | 204/196.11 |  |

See application file for complete search history.

(56) **References Cited**

U.S. PATENT DOCUMENTS

|             |         |                |
|-------------|---------|----------------|
| 2,944,957 A | 7/1960  | Keidel         |
| 3,009,865 A | 11/1961 | Mueller et al. |
| 3,072,128 A | 1/1963  | James          |
| 3,216,916 A | 11/1965 | Locke          |

FOREIGN PATENT DOCUMENTS

|    |              |        |       |            |
|----|--------------|--------|-------|------------|
| EP | 1640478 A2 * | 3/2006 | ..... | C23F 13/04 |
| JP | 2010-43307   | 2/2010 |       |            |

OTHER PUBLICATIONS

Derwent abstract for DE 2,217,715.\*  
 White et al (“Ice Houses and Ice Supply”, National Lumber Manufacturers Association, 1916, pp. “Ten”-“Eleven”) (Year: 1916).\*  
 “Moisture” by Oxford Dictionary. (Year: 2018).\*

\* cited by examiner



Fig. 1



Fig. 2



Fig. 3



Fig. 4

## 1

**CATHODIC PROTECTION FOR WOOD  
VENEER DRYERS AND METHOD FOR  
REDUCING CORROSION OF WOOD  
VENEER DRYERS**

TECHNICAL FIELD

The present invention relates generally to the protection of metallic structures or surfaces prone to corrosion and, in particular, this invention relates to cathodic protection for wood veneer dryers and methods for reducing corrosion of wood veneer dryers.

BACKGROUND OF INVENTION

Single and multiple deck conveyor dryers for reducing the moisture content of sheet materials, including green (or wet) wood veneer, wherein the material being dried is conveyed through a stationary drying chamber while heated gases are circulated through the drying chamber, are well-known in the art. Evaporation of moisture, inorganic compounds, and/or organic compounds (i.e. volatile organic compounds (V.O.C.'s)) from the material being dried causes a build-up of steam within the dryer, which may condense with carbon dioxide to form a corrosive liquid on the walls of the veneer dryer and on other equipment. Many metals corrode due to exposure to moisture and corrosion of metallic structures and surfaces of the dryer has been a major problem in the veneer drying art.

It is desirable to control the corrosion of metallic structures and surfaces of a wood veneer dryer to extend the lifetime of the dryer. To reduce corrosion, metallic structures and surfaces inside of veneer dryers may be made from or coated with corrosion-resistant alloys, such as stainless steel. However, corrosion-resistant alloys are typically expensive. Furthermore, moisture is not precluded from migrating into dryer panel cracks or missed welds not treated with the corrosion-resistant alloy. There is accordingly a need in the art for a wood veneer dryer wherein the metallic structures and surfaces inside the dryer susceptible to corrosion are protected.

Cathodic protection is known in the art to control the corrosion of a metal by making it the cathode of an electrolytic cell. The metal to be protected is connected to a more easily corroded "sacrificial" metal that acts as the anode. The sacrificial metal then corrodes instead of the protected metal. The driving force for the cathodic protection current is the difference in electrode potential between the anode and the cathode.

A cathodic protection system is essentially a closed electric circuit that requires an anode and cathode to be immersed in an electrolyte; hence, cathodic protection is not used to prevent atmospheric corrosion. Typically, the structure to be protected is immersed in a body of fresh or salt water or is buried in moisture-rich soil.

In practice, the main use of cathodic protection is to protect steel structures immersed in a body of water or buried in moisture-rich soil (for example, the exterior surfaces of pipelines, ships' hulls, jetties, foundation piling, steel sheet piling, offshore platforms, and the interior surfaces of water-storage tanks and water-circulating systems).

Due to high maintenance and installation costs, cathodic protection is typically considered to be prohibitively expensive for use with relatively small scale structures, such as wood veneer dryers. Use is further limited by the need for structures to be immersed in a body of water or buried in moisture-rich soil.

## 2

The foregoing examples of the related art and limitations related thereto are intended to be illustrative and not exclusive. Other limitations of the related art will become apparent to those of skill in the art upon a reading of the specification and a study of the drawings.

SUMMARY OF THE INVENTION

The following embodiments and aspects thereof are 10 described and illustrated in conjunction with systems, tools, and methods which are meant to be exemplary and illustrative, not limiting in scope. In various embodiments, one or more of the above-described problems have been reduced or 15 eliminated, while other embodiments are directed to other improvements.

One aspect of the present invention provides a cathodic protection system for use with a wood veneer dryer. The cathodic protection system includes a DC power supply and an anode mounted inside the veneer dryer in a position to be 20 electrolytically coupled to metallic structures or surfaces inside the veneer dryer when an electrolytic medium is present. The DC power supply has a positive pole electrically connected to the anode and a negative pole electrically connected to the metallic structures or surfaces inside the 25 veneer dryer.

In some embodiments, the anode is more electronegative than the metallic structures or surfaces.

In some embodiments, the anode comprises one or more of high silicon iron, graphite, mixed metal oxides, lead 30 alloys, platinum, zinc, aluminum, magnesium, cadmium, niobium, tantalum, titanium, ruthenium, ruthenium oxide, rhodium, and rhodium oxide, preferably niobium.

In some embodiments, the anode comprises a niobium ribbon.

In some other embodiments, the anode is coated with a 35 material that is more electronegative than the metallic structures and surfaces.

In some embodiments, the material comprises one or more of high silicon iron, graphite, mixed metal oxides, lead 40 alloys, platinum, zinc, aluminum, magnesium, cadmium, niobium, tantalum, titanium, ruthenium, ruthenium oxide, rhodium, and rhodium oxide, preferably niobium.

In some embodiments, the anode comprises a niobium-coated ribbon.

In some embodiments, the anode is wrapped in an air-permeable membrane.

In some embodiments, the air-permeable membrane comprises one or more of a mineral wool, glass fibers, ceramics, and clays, preferably mineral wool.

In some embodiments, the anode extends from an input 50 end to an output end of the veneer dryer inside a drying chamber.

In some embodiments, the cathodic protection system further includes a computer system to monitor the conditions 55 inside the veneer dryer and to adjust the amount of current supplied by the DC power supply based on the detected conditions.

In some embodiments, the DC power supply supplies an amount of current to the anode and metallic structures or 60 surfaces inside the veneer dryer to shift the potential of the metallic structures or surfaces within the range of about (-) 0.700 V vs. silver/silver chloride (Ag/AgCl) to about (-) 1.200 V vs. silver/silver chloride (Ag/AgCl), preferably about (-) 0.800 V vs. silver/silver chloride (Ag/AgCl) or about (-) 0.950 V vs. silver/silver chloride (Ag/AgCl).

In some other embodiments, the DC power supply supplies an amount of current to the anode and metallic struc-

tures or surfaces inside the veneer dryer based on one or more of pH, temperature, electrolytic medium concentration, and electrolytic medium conductivity.

In some embodiments, the electrolytic medium comprises a high-humidity atmosphere inside the veneer dryer.

In some embodiments, the anode is mounted in a protective housing inside the veneer dryer.

Another aspect of the present invention provides a method for reducing the corrosion of metallic structures or surfaces inside a wood veneer dryer. The method includes mounting an anode inside a veneer dryer in a position to be electrolytically coupled to the metallic structures or surfaces inside the veneer dryer when an electrolytic medium is present inside the veneer dryer. A positive pole of a DC power supply is electrically connected to the anode and a negative pole of the DC power supply is electrically connected to the metallic structures and surfaces. Green wood veneer is conveyed through the veneer dryer and heated to a temperature sufficient to produce a high-humidity atmosphere inside the veneer dryer. A controlled amount of current is supplied by the DC power supply to electrolytically couple the anode to the metallic structures or surfaces.

In some embodiments, the conditions inside the veneer dryer are monitored and the amount of current supplied by the DC power supply is adjusted based on the detected conditions.

In some embodiments, the amount of current supplied shifts the potential of the metallic structures or surfaces within the range of about (-) 0.700 V vs. silver/silver chloride (Ag/AgCl) to about (-) 1.200 V vs. silver/silver chloride (Ag/AgCl), preferably about (-) 0.800 V vs. silver/silver chloride (Ag/AgCl) or about (-) 0.950 V vs. silver/silver chloride (Ag/AgCl).

In some other embodiments, the amount of current supplied is ascertainable based on one or more of pH, temperature, electrolytic medium concentration, and electrolytic medium conductivity.

In some embodiments, the anode is wrapped in an air-permeable membrane.

In some embodiments, the air-permeable membrane comprises one or more of a mineral wool, glass fibers, ceramics, and clays, preferably mineral wool.

In some embodiments, the anode is more electronegative than the metallic structures or surfaces.

In some embodiments, the anode comprises one or more of high silicon iron, graphite, mixed metal oxides, lead alloys, platinum, zinc, aluminum, magnesium, cadmium, niobium, tantalum, titanium, ruthenium, ruthenium oxide, rhodium, and rhodium oxide, preferably niobium.

In some embodiments, the anode comprises a niobium ribbon.

In some other embodiments, the anode is coated with a material that is more electronegative than the metallic structures and surfaces.

In some embodiments, the material comprises one or more of high silicon iron, graphite, mixed metal oxides, lead alloys, platinum, zinc, aluminum, magnesium, cadmium, niobium, tantalum, titanium, ruthenium, ruthenium oxide, rhodium, and rhodium oxide, preferably niobium.

In some embodiments, the anode comprises a niobium-coated ribbon.

In some embodiments, the anode extends from an input end of the veneer dryer to an output end of a drying chamber of the veneer dryer.

In some embodiments, the anode is mounted in a protective housing inside the veneer dryer.

In addition to the exemplary aspects and embodiments described above, further aspects and embodiments will become apparent by reference to the drawings and by study of the following detailed descriptions.

## BRIEF DESCRIPTION OF DRAWINGS

Exemplary embodiments are illustrated in referenced figures of the drawings. It is intended that the embodiments and figures disclosed are to be considered illustrative of the invention rather than restrictive.

FIG. 1 is a schematic of a cathodic protection system according to an embodiment of the present invention.

FIG. 2 is a partial cross-sectional side elevation view of the cathodic protection system of the embodiment shown in FIG. 1.

FIG. 3 is a partial perspective view of a protective housing of the cathodic protection system shown in FIG. 1 mounted inside a dryer.

FIG. 4 is a partial perspective view of an anode of the cathodic protection system shown in FIG. 1.

## DETAILED DESCRIPTION

Throughout the following description specific details are set forth in order to provide a more thorough understanding to persons skilled in the art. However, well known elements may not have been shown or described in detail to avoid unnecessarily obscuring the disclosure. Accordingly, the description and drawings are to be regarded in an illustrative, rather than a restrictive, sense.

In this specification, the term "cathodic protection" means controlling the corrosion of a metal structure or surface by making it the cathode of an electrolytic cell. The term "electrolytic cell" means a cell consisting of an electrolyte, its container, and two electrodes (i.e. an anode and a cathode), in which a redox reaction between the electrodes and the electrolyte occurs when an electrical current is applied. The term "anode" means an electrode or terminal by which current enters an electrolytic cell. The term "cathode" means an electrode or terminal by which current leaves an electrolytic cell. The term "electrolyte" means a medium capable of conducting current and in which the flow of current is accompanied by the movement of ions. The term "electrolytically coupled" means the coupling of a pair of electrodes in an electrolytic cell through an electrolyte thereby producing a redox reaction when an electrical current is applied to the cell. The term "corrosive medium" means any fluid that is corrosive to, or promotes corrosion of, a metallic structure or surface. The term "electrolytic medium" means any fluid capable of conducting current and in which the flow of current is accompanied by the movement of ions. The term "moisture" means a fluid, including but not limited to steam and/or condensed steam. The term "high-humidity atmosphere" means an atmosphere having a relatively high amount of moisture. The term "input end" in relation to the wood veneer dryer and components thereof means the end wherein wood veneer to be dried is introduced into the dryer, input end seal chamber, drying chamber, intermediary chamber, or cooling chamber. The term "output end" in relation to the wood veneer dryer and components thereof means the end opposite to the input end, i.e. the end wherefrom dried wood veneer exits the dryer, input end seal chamber, drying chamber, intermediary chamber, or cooling chamber. The term "about" means near the stated value (i.e. within +/-10% of the stated value).

A cathodic protection system **10**, as shown in FIGS. **1** and **2**, comprises a wood veneer dryer **20**, an anode **30** mounted inside veneer dryer **20**, and an external DC power supply **40** having a positive pole **42** electrically connected to anode **30** and a negative pole **44** electrically connected to veneer dryer **20**. Veneer dryer **20** may be a conventional single or multiple deck conveyor dryer for reducing the moisture content of sheet materials, including green wood veneer, wherein the material being dried is conveyed from an input end **22** to an output end **24** of a stationary drying chamber **26** while heated gases are circulated through drying chamber **26**.

As the wood veneer to be dried is heated, moisture and inorganic and/or organic compounds (such as V.O.C.'s) are released from the wood veneer producing a high-humidity atmosphere inside veneer dryer **20**. The high-humidity atmosphere inside veneer dryer **20** serves as a corrosive medium and/or an electrolytic medium inside veneer dryer **20**. The composition of the corrosive medium and/or the electrolytic medium inside veneer dryer **20** will vary depending on the species of wood dried and the conditions found inside veneer dryer **20** (i.e. temperature, pH, humidity, etc.).

Referring to FIG. **2**, anode **30** is mounted inside veneer dryer **20** in a position to be electrolytically coupled to the metallic structures and/or surfaces inside veneer dryer **20** when an electrolyte is present. In some embodiments, anode **30** is mounted to a ceiling **28** of veneer dryer **20** and extends from input end **22** to output end **24** of drying chamber **26**. Positive pole **42** of DC power supply **40** is electrically connected to anode **30** at one or more locations along the length of anode **30** to supply current to anode **30**. For example, in some embodiments, positive pole **42** of DC power supply **40** may be electrically connected to anode **30** about every 4.5 to 6 m (15 to 20 feet) along the length of anode **30**.

In some embodiments, anode **30** may be more electro-negative than the metallic structures and surfaces inside veneer dryer **20**. Based on the conditions found within veneer dryer **20** (for example, temperature and/or pH), anode **30** may comprise one or more of the following materials: high silicon iron, graphite, mixed metal oxides, lead alloys, platinum, zinc, aluminum, magnesium, cadmium, niobium, tantalum, titanium, ruthenium, ruthenium oxide, rhodium, and rhodium oxide, preferably niobium. In some other embodiments, anode **30** may be coated with a material that is more electronegative than the metallic structures and surfaces inside veneer dryer **20**. Based on the conditions found within veneer dryer **20** (for example, temperature and/or pH), the coating may comprise one or more of the following materials: high silicon iron, graphite, mixed metal oxides, lead alloys, platinum, zinc, aluminum, magnesium, cadmium, niobium, tantalum, titanium, ruthenium, ruthenium oxide, rhodium, and rhodium oxide, preferably niobium. In some embodiments, anode **30** comprises a niobium-coated wire or a niobium-coated ribbon. In other embodiments, anode **30** comprises niobium or a niobium ribbon. Persons skilled in the art will recognize that anode **30** may be comprised of or coated with any material that exhibits any one or more of the following features: good electrical conduction; a low rate of corrosion; good mechanical properties; the ability to withstand the stresses which they may be subjected to during installation and in service; the ability to be readily fabricated into a variety of shapes; low cost; and/or the ability to withstand high current densities at its surface without forming resistive barrier oxide layers. Niobium, for example, can resist becoming passive (i.e. developing an oxidation layer) at high tempera-

tures and within the voltage range required to operate catalytic protection system **10**, while being capable of delivering constant watt density when a current is applied thereto in a closed circuit.

In some embodiments, as shown in FIG. **3**, anode **30** may be mounted to ceiling **28** of veneer dryer **20** inside a protective housing **36**. Protective house **36** is air- and moisture-permeable. Protective housing **36** may comprise one or more of steel, mild steel, stainless steel, and aluminum, preferably mild steel.

In some embodiments, as shown in FIG. **4**, anode **30** may be wrapped in an air-permeable membrane **34**. As wood veneer is dried and a high-humidity atmosphere is produced inside veneer dryer **20**, membrane **34** may become saturated with moisture and/or inorganic and/or organic compounds, whereby saturated membrane **34** may serve as an electrolytic medium inside veneer dryer **20**. In some embodiments, membrane **34** comprises mineral wool, glass fibers, ceramics, clays, or a combination thereof, preferably mineral wool. Persons skilled in the art will recognize that membrane **34** may comprise any suitably porous material capable of withstanding the high temperatures employed inside veneer dryer **20** and capable of producing an electrolytic medium when saturated by a high-humidity atmosphere.

In operation, DC power supply **40** supplies a controlled amount of current to electrolytically couple anode **30** and the metallic structures and/or surfaces inside veneer dryer **20** when an electrolytic medium is present inside veneer dryer **20**. The metallic structures and/or surfaces are thereby rendered the cathode of cathodic protection system **10** and protected from corrosion. For example, DC power supply **40** may use low voltage DC current to shift the potential of the metallic structures and/or surfaces inside veneer dryer **20** within the range of about (-) 0.700 V vs. silver/silver chloride (Ag/AgCl) to about (-) 1.200 V vs. silver/silver chloride (Ag/AgCl), preferably about (-) 0.800 V vs. silver/silver chloride (Ag/AgCl) or about (-) 0.950 V vs. silver/silver chloride (Ag/AgCl). Persons skilled in the art will recognize that the amount of current supplied by DC power supply **40** is readily ascertainable based on pH, temperature, the concentration of the electrolytic medium inside veneer dryer **20**, and/or the conductivity of the electrolytic medium inside veneer dryer **20**.

A computer system (not shown) may be used to monitor the conditions (such as temperature, pH, the concentration of the electrolytic medium, and/or the conductivity of the electrolytic medium) inside veneer dryer **20** and the current supplied by DC power supply **40** may be adjusted based on the detected conditions. The computer system thereby maintains an optimum current output over the life of anode **30**. In the event that cathodic protection system **10** fails to operate, the computer system may be used to notify a user.

#### INTERPRETATION OF TERMS

Unless the context clearly requires otherwise, throughout the description and the claims:

“comprise”, “comprising”, and the like are to be construed in an inclusive sense, as opposed to an exclusive or exhaustive sense; that is to say, in the sense of “including, but not limited to”;

“connected”, “coupled”, or any variant thereof, means any connection or coupling, either direct or indirect, between two or more elements; the coupling or connection between the elements can be physical, logical, or a combination thereof;

"herein", "above", "below", and words of similar import, when used to describe this specification, shall refer to this specification as a whole, and not to any particular portions of this specification; "or", in reference to a list of two or more items, covers all of the following interpretations of the word: any of the items in the list, all of the items in the list, and any combination of the items in the list; the singular forms "a", "an", and "the" also include the meaning of any appropriate plural forms.

Words that indicate directions such as "vertical", "transverse", "horizontal", "upward", "downward", "forward", "backward", "inward", "outward", "left", "right", "front", "back", "top", "bottom", "below", "above", "under", and the like, used in this description and any accompanying claims (where present), depend on the specific orientation of the apparatus described and illustrated. The subject matter described herein may assume various alternative orientations. Accordingly, these directional terms are not strictly defined and should not be interpreted narrowly.

Where a component (e.g. a substrate, assembly, device, manifold, etc.) is referred to above, unless otherwise indicated, reference to that component (including a reference to a "means") should be interpreted as including as equivalents of that component any component which performs the function of the described component (i.e., that is functionally equivalent), including components which are not structurally equivalent to the disclosed structure which performs the function in the illustrated exemplary embodiments described herein.

Specific examples of systems, methods, and apparatus have been described herein for purposes of illustration. These are only examples. The technology provided herein can be applied to systems other than the example systems described above. Many alterations, modifications, additions, omissions, and permutations are possible within the practice of this invention. This invention includes variations on described embodiments that would be apparent to the skilled addressee, including variations obtained by: replacing features, elements and/or acts with equivalent features, elements and/or acts; mixing and matching of features, elements and/or acts from different embodiments; combining features, elements and/or acts from embodiments as described herein with features, elements and/or acts of other technology; and/or omitting combining features, elements and/or acts from described embodiments.

It is therefore intended that the following appended claims and claims hereafter introduced are interpreted to include all such modifications, permutations, additions, omissions, and sub-combinations as may reasonably be inferred. The scope of the claims should not be limited by the preferred embodiments set forth in the examples, but should be given the broadest interpretation consistent with the description as a whole.

We claim:

1. A cathodic protection system for use with a wood veneer dryer, the cathodic protection system comprising:  
the wood veneer dryer;  
an anode mounted inside the wood veneer dryer in a position to be electrolytically coupled to metallic structures or surfaces inside the veneer dryer when an electrolytic medium is present inside the veneer dryer; and  
a DC power supply having a positive pole electrically connected to the anode and a negative pole electrically connected to the metallic structures or surfaces, wherein: 65

the anode is comprised of or coated with one or more of high silicon iron, graphite, mixed metal oxides, platinum, niobium, tantalum, ruthenium, ruthenium oxide, rhodium, and rhodium oxide, and

the anode is wrapped in an air-permeable membrane capable of producing the electrolytic medium when saturated by a high-humidity atmosphere inside the dryer.

2. The cathodic protection system according to claim 1, 10 wherein the anode comprises niobium.

3. The cathodic protection system according to claim 2, wherein the anode comprises a niobium ribbon.

4. The cathodic protection system according to claim 1, 15 wherein the air-permeable membrane comprises one or more of a mineral wool, glass fibers, ceramics, and clays.

5. The cathodic protection system according to claim 4, wherein the air-permeable membrane comprises mineral wool.

6. The cathodic protection system according to claim 1, 20 wherein the anode extends from an input end to an output end of the veneer dryer inside a drying chamber.

7. The cathodic protection system according to claim 1, 25 further comprising a computer system to monitor the conditions inside the veneer dryer and adjust the amount of current supplied by the DC power supply based on the detected conditions.

8. The cathodic protection system according to claim 1, 30 wherein the DC power supply supplies an amount of current to the anode and metallic structures or surfaces inside the veneer dryer to shift the potential of the metallic structures or surfaces within the range of about (-) 0.700 V vs. silver/silver chloride (Ag/AgCl) to about (-) 1.200 V vs. silver/silver chloride (Ag/AgCl).

9. The cathodic protection system according to claim 8, 35 wherein the DC power supply supplies an amount of current to the anode and metallic structures or surfaces inside the veneer dryer to shift the potential of the metallic structures or surfaces to about (-) 0.800 V vs. silver/silver chloride.

10. The cathodic protection system according to claim 8, 40 wherein the DC power supply supplies an amount of current to the anode and metallic structures or surfaces inside the veneer dryer to shift the potential of the metallic structures or surfaces to about (-) 0.950 V vs. silver/silver chloride.

11. The cathodic protection system according to claim 1, 45 wherein the DC power supply supplies an amount of current to the anode and metallic structures or surfaces inside the veneer dryer based on one or more of pH, temperature, electrolytic medium concentration, and electrolytic medium conductivity.

12. The cathodic protection system according to claim 1, 50 wherein the anode is mounted in a protective housing inside the veneer dryer.

13. A method for reducing the corrosion of metallic structures or surfaces inside a wood veneer dryer, the 55 method comprising:

mounting an anode inside the wood veneer dryer in a position to be electrolytically coupled to the metallic structures or surfaces inside the veneer dryer when an electrolytic medium is present inside the veneer dryer, wherein the anode is comprised of or coated with one or more of high silicon iron, graphite, mixed metal oxides, platinum, niobium, tantalum, ruthenium, ruthenium oxide, rhodium, and rhodium oxide;

electrically connecting a positive pole of a DC power supply to the anode and electrically connecting a negative pole of the DC power supply to the metallic structures or surfaces;

conveying wood veneer through the veneer dryer and heating the wood veneer inside the veneer dryer to a temperature sufficient to produce a high-humidity atmosphere inside the veneer dryer; and supplying a controlled amount of current to electrolytically couple the anode to the metallic structures or surfaces, wherein the anode is wrapped in an air-permeable membrane capable of producing the electrolytic medium when saturated by the high-humidity atmosphere inside the dryer.

**14.** The method according to claim **13**, further comprising monitoring the conditions inside the veneer dryer and adjusting the amount of current supplied by the DC power supply based on the detected conditions.

**15.** The method according to claim **13**, wherein the amount of current supplied shifts the potential of the metallic structures or surfaces within the range of about (-) 0.700 V vs. silver/silver chloride (Ag/AgCl) to about (-) 1.200 V vs. silver/silver chloride (Ag/AgCl).

**16.** The method according to claim **15**, wherein the amount of current supplied shifts the potential of the metallic structures or surfaces to about (-) 0.800 V vs. silver/silver chloride.

**17.** The method according to claim **15**, wherein the amount of current supplied shifts the potential of the metallic structures or surfaces to about (-) 0.950 V vs. silver/silver chloride.

**18.** The method according to claim **13**, wherein the amount of current supplied is ascertainable based on one or more of pH, temperature, electrolytic medium concentration, and electrolytic medium conductivity.

**19.** The method according to claim **13**, wherein the air-permeable membrane comprises one or more of a mineral wool, glass fibers, ceramics, and clays.

**20.** The method according to claim **19**, wherein the air-permeable membrane comprises mineral wool.

**21.** The method according to claim **13**, wherein the anode comprises niobium.

**22.** The method according to claim **21**, wherein the anode comprises a niobium ribbon.

**23.** The method according to claim **13**, wherein the anode extends from an input end of the veneer dryer to an output end of a drying chamber of the veneer dryer.

**24.** The method according to claim **13**, wherein the anode is mounted in a protective housing inside the veneer dryer.

\* \* \* \* \*